

1

3,251,872

HARD ACID WAXES POOR IN PARAFFINS AND  
PROCESS FOR THEIR MANUFACTURE

Josef Kaupp and Oswald Metz, Gersthofen, near Augsburg, Germany, assignors to Farbwurke Hoechst Aktiengesellschaft vormals Meister Lucius & Brüning, Frankfurt am Main, Germany, a corporation of Germany

No Drawing. Filed Sept. 26, 1961, Ser. No. 140,696

Claims priority, application Germany, Sept. 28, 1960,

F 32,214

4 Claims. (Cl. 260—451)

The present invention relates to a process for the manufacture of hard acid waxes which are poor in paraffins.

It is known to transform high molecular weight aliphatic hydrocarbons into acid waxes by chlorinating, dehydrochlorinating and oxidizing the olefins with chromic acid. The simple oxidation performed in this known process with chromic acid yields, however, acid waxes which have an insufficient hardness, above all when a low paraffin content is desired, so that further process steps are required. These further steps relate to the extraction of the low molecular weight portions, or isolation of the carboxylic acids by saponification, extraction of the unsaponifiable matter, and decomposition of the soaps with mineral acids. It is complicated to conduct these processes and, furthermore, it is not economical to produce acid waxes from hard paraffins in this manner.

Moreover, synthetic paraffins having a solidification point of about 50° C. can be transformed into high molecular weight paraffin-containing fatty acids by the addition of 0.6 to 0.7 mol of chlorine on one mol of paraffin, subsequent dehydrochlorination and repeated treatment with a solution of concentrated sulfuric acid and sodium bicarbonate. The oxidation products thus obtained are suitable as impregnating agents for fibrous materials. They represent soft substances which cannot be used for manufacture of hard waxes.

It has now been found that hard acid waxes poor in paraffins can be obtained by chlorinating and dehydrochlorinating paraffins and oxidizing the olefins with chromic acid, when high molecular weight paraffin hydrocarbons having a solidification point above 90° C., and preferably above 95° C., are chlorinated in known manner to such an extent that more than 0.7 mol of chlorine is contained in the molecule, dehydrochlorinated in known manner and the olefins obtained are repeatedly oxidized with chromic acid until practically all double bonds have disappeared.

As starting materials there are suitable, for example, hard paraffins from the catalytic hydrogenation of carbon oxide, especially those having a solidification point above 95° C., or wax-like homo- or copolymers of ethylene or propylene having a medium molecular weight above 700, preferably above 800 and below 20,000, prepared by the so-called low pressure or high pressure synthesis, or mixtures of hard paraffins and the aforesaid wax-like olefin polymers. Still further, there can be used well refined paraffins obtained from crude oil or petroleum, provided that their solidification point is higher than 90° C. It is necessary to use paraffin hydrocarbons having very long chains since in the substitution the chlorine is statistically distributed over the whole paraffin molecule and in the oxidation the carbon chain breaks at the point where the chlorine was bound. The loss in hardness caused by the decomposition is the greater the lower the molecular weight of the starting paraffin.

The hardness of the acid waxes depends, in the first place, on the size of the molecules of the carboxylic acids and their paraffin content depends on the degree of

2

chlorination. The best products could be obtained if the chlorination with as little as 0.5 mol of chlorine per mol of paraffin would be complete, with fairly terminal substitution. The chlorination involves, however, the statistical substitution and multiple substitution. This multiple substitution mainly results from the fact that the long-chain paraffin molecules are attacked first. With an increasing degree of chlorination the solidification point of the unmodified paraffin descends, which means, however, that the average molecular weight of the residual paraffin portion diminishes. The largest molecules undergo multiple substitution in the first place. The multiple substitution commences already when less than half of all paraffin molecules is chlorinated. This involves a further reduction of the hardness in the oxidation due to manifold breakages of the chain. For these reasons, in the process of the present invention the maximum hardness of the acid waxes is bound to a minimum paraffin content, which can be the lower the higher the medium molecular weight of the hydrocarbons and the more uniform the hydrocarbons with respect to their chain lengths.

Owing to the occurrence of the multiple substitution more than 0.7 mol of chlorine must be introduced into each mol of paraffin for obtaining acid waxes which are poor in paraffins. When synthetic hard paraffins are chlorinated it is very advantageous to introduce 0.9–1.5 mols of chlorine into one mol of paraffin. Higher amounts of chlorine can be introduced when the molecular weight of the starting material is very high, as is the case with wax-like olefin polymers. The chlorination is carried out in known manner, generally by introducing gaseous chlorine, for example, into the melt, solution or suspension of the starting material. The dehydrochlorination is likewise carried out in known manner, for example thermically in the melt at a temperature in the range from 250° C.–350° C., if desired with the addition of substances promoting the separation of hydrogen chloride, such, for example, as bleaching earth, active carbon, lime, zinc dust or zinc oxide.

The olefins obtained after the dehydrochlorination are oxidized with chromosulfuric acid solutions of known composition in a manner such that the molten olefins are repeatedly oxidized, each time with a fresh chromosulfuric acid solution, while thoroughly mixing. The total amount of oxidant and the number of oxidations required are suitably determined by a previous test for each type of paraffin and degree of chlorination.

It is not expedient, of course, to use too high an amount of chromic acid; in general it is absolutely sufficient to use at most 300% of chromic acid, calculated on the weight of the dehydrochlorination product. As compared with a single oxidation with a large amount of chromic acid, the repeated application of smaller and always fresh amounts of chromic acid has the advantage that the olefins are more completely oxidized. This is perceptible by the reduction of the paraffin content of the oxidation products. Moreover, the hardness of the acid waxes is distinctly improved. The higher consumption of chromic acid unexpectedly does not increase the degree of oxidation, expressed by the acid number and saponification number, but serves exhaustively to oxidize the olefins and to improve the hardness.

The process of the invention enables high molecular weight paraffin hydrocarbons to be transformed in simple manner into hard acid waxes which are poor in paraffins by oxidizing the olefins with chromic acid without further processing. The acid waxes thus obtained are white or ivory-colored. Owing to their hardness and high flowing/dropping point they are suitable, for example, as acid components of high melting ester and amide waxes. For waxes of this kind there can be used as alcohol com-

ponent above all polyols, such, for example, as ethylene glycol, butylene glycol, hexane diol, glycerol, pentaerythritol, and as amine component above all di- and polyamines, such for example, as ethylene diamine, propylene diamine, hexamethylene diamine, dipropylene triamine, benzidine, 4,4'-diaminodiphenylmethane and the hydrogenation products thereof. The acids can be wholly or

In the following table there are given the characteristics of the three oxidation products. The flowing/dropping point and the penetrometer hardness (100 grams load, 5 seconds, 25° C.) were determined according to DIN 1995 and the paraffin content was determined by chromatography.

| Oxidation product | Number of oxidations | Consumption of CrO <sub>3</sub> , percent | Acid number | Saponification number | Flow point, drop point, °C. | Penetrometer hardness | Paraffin content, percent |
|-------------------|----------------------|-------------------------------------------|-------------|-----------------------|-----------------------------|-----------------------|---------------------------|
| I                 | 1                    | 185                                       | 122         | 143                   | 100.5/101.0                 | 4                     | 19.0                      |
| II                | 2                    | 190                                       | 109         | 129                   | 100.0/100.5                 | 2                     | 17.5                      |
| III               | 3                    | 250                                       | 111         | 126                   | 99.5/100.0                  | <0.5                  | 15.0                      |

partially transformed into soaps, for example of the alkali metals and/or alkaline earth metals, if desired after previous esterification.

The following examples serve to illustrate the invention but they are not intended to limit it thereto:

#### Example 1

A high molecular weight hard paraffin originating from the catalytic hydrogenation of carbon oxide and having a solidification point of 98° C. (according to ASTM D938-49) and a medium molecular weight (according to Rast) of 750 was chlorinated to a chlorine content of 9.0% (about 1 mol) and then dehydrochlorinated at 320° C.

500 grams of the dehydrochlorination product were oxidized once, for 4 hours at 110°-120° C., while stirring, with 200% of CrO<sub>3</sub>, calculated on the olefin, in the form of an aqueous chromosulfuric acid solution containing per liter about 520 grams of sulfuric acid and 110 grams of CrO<sub>3</sub>. 185% of CrO<sub>3</sub> were consumed.

#### Example 2

A high molecular weight hard paraffin from the catalytic carbon oxide hydrogenation having a solidification point of 101° C. and a medium molecular weight of 820 was chlorinated to a chlorine content of 7.5% (about 0.9 mol) and then dehydrochlorinated at 320° C.

25 500 grams of the dehydrochlorination product were oxidized once for 6 hours as described in Example 1 with 180% of CrO<sub>3</sub>. 155% of CrO<sub>3</sub> were consumed (oxidation product I).

500 grams of the dehydrochlorination product were oxidized twice for 4 hours as described in Example 1, each time with 120% of CrO<sub>3</sub>. A total amount of 152% of CrO<sub>3</sub> was consumed (oxidation product II).

Oxidation product II was then again oxidized as de-

scribed in Example 1 for 4 hours with 100% of CrO<sub>3</sub>. 60% of CrO<sub>3</sub> were consumed (oxidation product III).

35 The total consumption of CrO<sub>3</sub> in the triple oxidation thus amounted to 212%.

| Oxidation product | Number of oxidations | Consumption of CrO <sub>3</sub> , percent | Acid number | Saponification number | Flow point, drop point, °C. | Penetrometer hardness | Paraffin content, percent |
|-------------------|----------------------|-------------------------------------------|-------------|-----------------------|-----------------------------|-----------------------|---------------------------|
| I                 | 1                    | 155                                       | 105         | 130                   | 100.0/100.5                 | 4                     | 18.0                      |
| II                | 2                    | 152                                       | 101         | 114                   | 101.5/102.0                 | 3                     | 15.5                      |
| III               | 3                    | 212                                       | 116         | 130                   | 100.5/101.0                 | 1.5                   | 12.5                      |

After the removal of the consumed chrome salt solution, the oxidation product was washed with dilute sulfuric acid until it was free from chromic salts and then with water until it was free from acid, and dried (oxidation product I).

50 500 grams of the dehydrochlorination product were oxidized for 4 hours at 110°-120° C. while stirring with 120% of CrO<sub>3</sub>, calculated on the olefin. 105% of CrO<sub>3</sub> were consumed. After the removal of the exhausted chromic acid solution, the product was again oxidized in the same manner with 120% of CrO<sub>3</sub>. After 4 hours 85% of CrO<sub>3</sub> were consumed. A sample of the oxidation product was washed with dilute sulfuric acid until it was free from chromic salts and then with water until it was free from acid, and dried (oxidation product II).

The principal amount of the oxidation product was oxidized once more for 4 hours with 100% of CrO<sub>3</sub>. 60% of CrO<sub>3</sub> were consumed (oxidation product III). The total consumption of CrO<sub>3</sub> amounted to 250%, calculated on the olefin used.

When oxidation product III was reacted with the equivalent amount of 4,4'-diaminodicyclohexylmethane at 170° C.-180° C. an amidation product was obtained having a melting point of about 165° C.

#### Example 3

55 A wax-like low pressure polyethylene having a medium molecular weight of about 2,600, a solidification point of 109° C. and a melting point of 115° C. was chlorinated to a chlorine content of 7% (about 2.5 mols) and then dehydrochlorinated at 320° C.

60 500 grams of the dehydrochlorination product were oxidized once for 6 hours as described in Example 1 with 220% of CrO<sub>3</sub>. 200% of CrO<sub>3</sub> were consumed (oxidation product I).

65 500 grams of the dehydrochlorination product were oxidized three times as described in Example 1, each time with 100% of CrO<sub>3</sub> for 4 hours. A total amount of 220% of CrO<sub>3</sub> was consumed (oxidation product II).

| Oxidation product | Number of oxidations | Consumption of CrO <sub>3</sub> , percent | Acid number | Saponification number | Flow point, drop point, °C. | Penetrometer hardness | Paraffin content, percent |
|-------------------|----------------------|-------------------------------------------|-------------|-----------------------|-----------------------------|-----------------------|---------------------------|
| I                 | 1                    | 200                                       | 100         | 115                   | 108.0/108.5                 | 3.5                   | 6.8                       |
| II                | 3                    | 220                                       | 113         | 117                   | 108.0/108.5                 | 2.0                   | 5.5                       |

We claim:

1. A process for the manufacture of hard acid waxes which are poor in paraffins from high molecular weight paraffin hydrocarbons which comprises chlorinating a high molecular weight paraffin hydrocarbon having a solidification point above 90° C. to a chlorine content of more than 0.7 mol of chlorine in each mol of paraffin, dehydrochlorinating the chlorinated product to obtain an olefin, oxidizing said olefin for a period of 4-6 hours at a temperature of 110°-120° C. with chromic acid in an amount of 180-220% by weight of the dehydrochlorination product, removing the chromic acid solution, washing the oxidized olefin with dilute sulfuric acid, washing the oxidized olefin with water, and repeating the oxidation of the oxidized olefin three times using 100-120% of chromic acid by weight of the olefin in each of the said three oxidations, said oxidations removing substantially all of the double bonds of said olefin.

2. The process of claim 1 wherein hard paraffins originating from catalytic carbon oxide hydrogenation and having a solidification point above 95° C. are used as the high molecular weight paraffin hydrocarbons.

3. The process of claim 1 wherein waxy olefin polymers having a medium molecular weight of 700 to 20,000 are used as high molecular weight paraffin hydrocarbons.

4. A hard acid wax which is poor in paraffins obtained

5

10

15

from a high molecular weight paraffin hydrocarbon by chlorinating a high molecular weight paraffin hydrocarbon having a solidification point above 90° C. to a chlorine content of more than 0.7 mol of chlorine in each mol of paraffin, dehydrochlorinating the chlorinated product to obtain an olefin, oxidizing said olefin for a period of 4-6 hours at a temperature of 110-120° C. with chromic acid in an amount of 180-220% by weight of the dehydrochlorination product, removing the chromic acid solution, washing the oxidized olefin with dilute sulfuric acid, washing the oxidized olefin with water, and repeating the oxidation of the oxidized olefin three times using 100-120% of chromic acid by weight of the olefin in each of the said three oxidations, said oxidations removing substantially all of the double bonds of said olefin.

#### References Cited by the Examiner

##### UNITED STATES PATENTS

|           |        |                |         |
|-----------|--------|----------------|---------|
| 2,795,596 | 6/1957 | Kolling et al. | 260-450 |
| 2,835,691 | 5/1958 | Sauter         | 260-451 |
| 2,892,877 | 6/1959 | Kolling et al. | 260-450 |

25 LEON ZITVER, *Primary Examiner.*

ALPHONSO D. SULLIVAN, *Examiner.*